

1

3,281,221

## TIN PLATE IDENTIFICATION

Andy A. Denuzzio, Aliquippa, Pa., assignor to Jones & Laughlin Steel Corporation, Pittsburgh, Pa., a corporation of Pennsylvania  
No Drawing. Filed Feb. 28, 1964, Ser. No. 348,272  
8 Claims. (Cl. 29—191)

This invention relates to tin plate which is positively identified as to source. It is more particularly concerned with tin plate which is marked or branded in such a way that the marking is normally invisible, but can be discovered by stripping off the tin plate or the tin coating together with the tin-iron alloy layer.

Tin plate is commercially produced by steel manufacturers and is sold principally to manufacturers of tin cans. The tin cans in turn are sold to packers of foods of various kinds. The tin plate is shipped to the can manufacturer in the form of sheets or of coils and is cut up by him into can body blanks and can end blanks which he then fabricates into tin cans. The tin surface of both the body blanks and the end blanks must be free of all foreign substances as otherwise the food packed in the cans could be contaminated. Although the tin plate received by the can maker is identified as to source, this identification does not carry over to the body blanks and end blanks stamped therefrom. Consequently, although the cans shipped to a packer are identified as to the can fabricator, they are not identified as to the maker of the tin plate. Therefore, prior to my invention to be described, if canned food spoiled because of defective tin plate, there was no certainty of identifying the tin plate as being the product of one supplier if the can maker used tin plate from several sources, as is generally the case.

It is an object of my invention, therefore, to produce tin plate which carries a mark indicative of its source even when it is cut up and fabricated into cans. It is another object to provide such tin plate having an identifying mark which is visible only when the tin coating or the tin coating and the tin-iron alloy layer are removed. Other objects will appear in the course of the description of my invention which follows.

The tin plate of my invention comprises the conventional thin still base having the conventional tin coating which may be applied electrolytically or by hot dipping. Electrolytic tin plate is conventionally flow brightened, that is, heated briefly to a temperature slightly above the melting point of tin to flow the matte tin deposit, and then quenched. Both types of conventional tin plate are, therefore, heated above the melting point of tin during their manufacture, and this heating brings about an alloying of the tin and iron at the tin-iron interface which is visible under the microscope as a thin layer of this alloy intermediate the tin and iron. The surface of the steel base of the preferred tin plate of my invention is chemically treated prior to tinning so as to etch the steel base to a slight degree. This etching, which is clearly visible against the steel base, does not deleteriously affect the adherence of the tin thereto or the formation of tin-iron alloy between base and tin coating when the tin plate is heated. However, the appearance of the tin-iron alloy in the etched areas is different from that in the unetched areas of the base. As the tin-iron alloy is covered by the tin coating, the tin plate, as it leaves the tin pot or the flow brightener of an electro-tinning line, displays no evidence of the etching that has taken place. However, if the tin is stripped from the tin plate, the tin-iron alloy, which then becomes visible, displays a marking corresponding to the etched area of the base beneath it. If the tin-iron alloy is also stripped, the steel base displays the

2

mark produced by the etching. I prefer to apply the chemical to the steel base of my tin plate in an over-all pattern such that a plurality of repeats will appear on each can body blank and each can end blank which may be stamped therefrom. Thus, if a can made from tin plate of my invention proves defective, the supplier of the tin plate can be identified by cutting a sample from the can and stripping the tin or the tin and the tin-iron alloy therefrom.

As the great bulk of the tin plate now being sold is tinned electrolytically, I shall first describe the manufacture of my tin plate in that context. I apply my chemical etchant to the surface of the steel strip after the strip has been cleaned but prior to its entrance into the electro-tinning bath. Preferably, the chemical is applied by a rubber roller, the surface of which is cut out or embossed into the desired pattern. Etching begins immediately, but stops when the etchant is washed off by the bath solution into which the strip passes. In the electro-plating bath, tin is plated onto the strip in the conventional manner, the etching being insufficient to result in any change of external appearance of the deposited tin. I prefer to use the so-called halogen electrolyte of U.S. Patent 2,407,579 granted to E. W. Schweikher on September 10, 1946. When the strip is flow brightened, the heating affects the tin-iron alloy layer formed thereby so that its appearance over those etched areas is different from its appearance over unetched areas. The external surface of the brightened tin plate shows no marking at all.

In the manufacture of hot dipped tin plate, I apply my chemical etchant to the steel just before it enters the tin bath. Etching begins immediately, but I find that the steel is in the bath such a short time that the etching does not interfere with the adherence of the tin to the steel. As in the case of the electro-tinned steel, the etching also affects the appearance of the tin-iron alloy layer above the etched area, but does not mark the tin coating.

My preferred etchant is an 8% to 12% aqueous solution of ferric chloride. Those skilled in the art will have knowledge of other etchants that will produce the same effect.

My preferred new tin plate produced as I have here described, comprises therefor a steel base having an etched marking thereon which contrasts with its background—the base, a tin-iron alloy layer in immediate contact with the steel base, that layer also having a marking thereon which contrasts with its background—the tin-iron alloy layer, and a reflowed tin coating which exhibits no marking. The marking on the tin-iron alloy is immediately above the corresponding marking on the base. When the tin coating is stripped from my tin plate, which may be accomplished by known methods, the marking on the tin-iron alloy layer contrasts with its background and is clearly visible. When the tin-iron alloy layer is also stripped from my tin plate, which may also be accomplished by known methods, the marking on the steel base contrasts with its background and is clearly visible.

I claim:

1. A new article of manufacture comprising tin plate having on the steel base an etched mark which contrasts with its background so as to be clearly visible thereagainst when the tin coating is stripped therefrom.
2. The article of claim 1 in which the etched mark is a chemically etched mark.
3. The article of claim 1 in which the mark is invisible beneath the tin coating.
4. The article of claim 2 in which the chemically etched mark is the reaction product of the steel base and ferric chloride.
5. A new article of manufacture comprising tin plate having a tin-iron alloy layer intermediate the steel base and tin coating and having on the steel base an etched

mark which contrasts with its background so as to be clearly visible thereagainst when the tin coating and tin-iron alloy layer are stripped therefrom.

6. The article of claim 5 in which the tin plate is electrotinned and flow-brightened tin plate.

7. The article of claim 6 in which the electrotinned tin plate is halogen electrolyte tin plate.

8. A new article of manufacture comprising tin plate having a tin-iron alloy layer intermediate the steel base and tin coating and having on the steel base an etched mark and on the tin-iron alloy layer a corresponding mark immediately above the etched mark and occasioned thereby, which corresponding mark contrasts with its

background so as to be clearly visible thereagainst when the tin coating is stripped from the tin plate.

**References Cited by the Examiner**

UNITED STATES PATENTS

2,738,897 3/1956 Russell et al. \_\_\_\_\_ 29—196.4  
2,770,872 11/1956 Kadell \_\_\_\_\_ 29—196.4  
3,074,154 1/1963 Pearson et al. \_\_\_\_\_ 29—196.4

10 DAVID L. RECK, *Primary Examiner.*

HYLAND BIZOT, *Examiner.*

R. O. DEAN, *Assistant Examiner.*